

1,377,960.

H. K. DODGE,  
ANTISLIPPING TILE,  
APPLICATION FILED APR. 29, 1918.

Patented May 10, 1921.



*Fig. 1.*



*Fig. 2.*

INVENTOR

HERBERT K. DODGE

*Clayton L. Jenkins*  
BY  
ATTORNEY

Witnesses

L. F. Butterfield  
P. Q. Sessions

# UNITED STATES PATENT OFFICE.

HERBERT K. DODGE, OF PALISADES, NEW JERSEY, ASSIGNOR TO NORTON COMPANY,  
A CORPORATION OF MASSACHUSETTS.

## ANTISLIPPING TILE.

1,377,960.

Specification of Letters Patent. Patented May 10, 1921.

Application filed April 29, 1918. Serial No. 231,417.

To all whom it may concern:

Be it known that I, HERBERT K. DODGE, a citizen of the United States of America, residing at Palisades, in the county of Bergen and State of New Jersey, have invented 5 certain new and useful Improvements in Antislipping Tiles, of which the following is a full, clear, and exact specification.

My invention relates to safety treads and 10 more particularly to anti-slipping tread blocks or tiles having a high surface coefficient of friction and great resistivity to footwear.

Owing to the frequent accidents caused 15 by persons slipping on stairways and public walks made of wood, brick, paving stone, concrete, etc., numerous attempts have been made, as by forming the treads with corrugated or discontinuous surfaces, to render 20 such materials safe for pedestrians, but heretofore no tread has been found capable of retaining its anti-slipping characteristics and original form where exposed to the constant wear of pedestrian traffic.

25 The anti-slipping properties of the extremely hard abrasive materials have been recognized and flooring and paving construction experts have attempted to provide safety treads by incorporating such abrasives in artificial blocks or stones. For example, small amounts of isolated abrasive grains have been embedded in various substances, such as asphalt, rubber and other organic bodies which produce a fire hazard, 30 or in lead or cements, such as magnesium oxychlorid or concrete. Such enveloping substances have little durability or poor adhesion to the abrasive grains, hence where the body of the tread is exposed to wear,

35 the grains are soon loosened from their settings and the utility of the tread impaired. To overcome this objection, tread strips made of lead or cement containing abrasive are set in grooved metal frames, but the 40 safety tread portion wears away and leaves the smooth iron of the frame exposed and thus endangers the pedestrian. Moreover, such tread constructions require that the nose of a stair be made of metal, which is 45 smooth, whereas the stair edge should have the maximum anti-slipping characteristics. Similarly, abrasive grains have been cast in the tread portions of iron blocks, but these 50 soon wear out and the tread blocks become 55 smooth and slippery metal surfaces.

I have discovered, on the other hand, that a safety tread which will be permanently wear-resisting and safe for pedestrians may be made in the form of a tile of durable, anti-slipping, granular material constituting 60 the major portion of the tread volume, and bonded together by a medium capable of uniting them integrally into a wear-resisting structure, as distinguished from a body in which isolated grains are embedded. 65

With these features in mind, one object 70 of my invention is to provide a unitary tread block which in itself is tough, hard and of high tensile strength, which resists footwear to a high degree and has a long life of utility and which retains a rough friction surface under all conditions of normal pedestrian wear.

A further object of my invention is to 75 utilize durable, granular abrasive materials and make a safety tread therefrom and to bond together such grains of desired anti-slipping characteristics by a ceramic material which is capable of uniting intimately therewith and forming an integral, wear-resisting tile body, in which the abrasive granules constitute the major portion of the tread volume and receive substantially 80 all of the traffic wear.

A still further object is to provide a plane 85 surfaced safety tile of simple design and of uniform appearance and composition, which may be manufactured in quantities and laid in position like ordinary flooring tiles to cover those areas which are most 90 exposed to wear, without the necessity for supplemental reinforcements appearing on the tread surface.

With these and other objects in view as 95 will appear from the following disclosure, my invention resides in the construction and the composition herein described and covered by the appending claims.

Referring to the drawings, in which like 100 numerals indicate like parts:

Figure 1 is a perspective view of one form of tile; and

Fig. 2 is a diagrammatic section of my tile 105 embedded in concrete on the edge of a railroad platform.

In the practice of my invention, I bond 110 hard, anti-slipping and wear-resisting granular material into a desired shape by means of a bonding substance which is durable and capable of holding the grains in place un-

der all normal usages of pedestrian traffic and yet of breaking away ultimately to present fresh cutting grains on the surface when the old ones have become worn and 5 dulled. Of the various hard materials suitable for safety treads which I may utilize, I find it desirable to employ those which have a hardness of 9 or more on Mohs's scale, where traffic wear conditions are 10 severe. As a specific example of such a wear-resisting, anti-slipping material which is harder than 9, crystalline grains in which alumina is the main ingredient may be mentioned.

15 To prepare a tile of such hard granular material, I bond the grains together with a suitable substance capable of giving the block the desired tensile strength, toughness and wearing qualities. For this purpose I 20 have found most satisfactory a ceramic bond which may be vitrified or fused to a glassy condition around the granular particles and then solidified into a magma tenaciously adhering to the grains and binding 25 them together into a compact unitary mass. I preferably employ a vitrifiable glass fusing ceramic bond, such as a low fusing clay material, comprising for example feldspar mixed with slip clay and ball clay. Such a 30 clay bond during its state of fusion effects an exceedingly intimate union with the surface of the anti-slipping material. Where aluminum oxid is the main ingredient of 35 the hard granules, the fused clay material has a dissolving action upon the surface of the oxid grain, whereby the structure becomes substantially homogeneous and the grains are held firmly in place. It is often 40 found that the vitreous magma is filled with sillimanite needles interlaced between the surfaces of the alumina crystals, this structure accounting in part for the hardness and durability of the bond.

45 The tile may be made in accordance with approved ceramic methods. The nature of the bond and the proportions of the ingredients depend upon the type and the sizes of the abrasive grains as well as the firing and 50 other operations employed, it being understood that a ceramic article of this type consists mainly of hard grains and that the bond is contained largely in the voids between the grains but does not fill them; hence one ordinarily employs only sufficient 55 bond to give the desired physical characteristics, with the dangers of swelling and of the bond strength being too weak as the usual limiting factors in determining the 60 correct proportions. As a specific example of one satisfactory composition made up of feldspar, slip clay and ball clay to be treated as hereinafter described, I may form a tile of 77% by weight of crystalline alumina 65 grains and 23% of bond. These materials

may be mixed in dry form; then after wetting the mixture sufficiently so that it will retain its shape, it is preferably subjected to high pressure in a steel mold of a desired form to make the mass dense and 70 compact. Since the block in this condition has no strength or wearing qualities, it is first dried and then fired or burned in a suitable ceramic kiln, at a temperature around 1300° C., depending upon the specific nature of the ingredients used, to produce a glassy condition in the bond. The burning is conducted slowly so as not to destroy the ware, the operation lasting, for example, 100 hours, after which the tile is 80 cooled slowly for a similar length of time.

By this means I produce a ceramic tile, unlike a block of glass or porcelain containing hard grains embedded therein, but in which granular particles, comprising previously molten alumina, for example, are bonded by a glassy ceramic material into a dense, porous body, which in the specific example given above, has a porosity of about 30% and a water absorption of about 15%. The alumina grains, which constitute the major portion of the body, are drawn together into a dense mass by the shrinkage of the ceramic material when fused. This vitreous substance forms bonding posts, as it were, between adjacent grain surfaces and leaves spaces interspersed therebetween, thus permitting a large part of the grain surface to be exposed as well as providing sharp edged pores to assist in forming a 90 safety tread.

95 Alumina, to be sufficiently hard for my purposes must be in a crystalline form. While the impure forms of crystalline alumina, such as emery and corundum which contain various proportions of other ingredients, may be utilized, I preferably employ an artificial substance prepared for example by melting alumina, bauxite, or 100 other alumina containing material in an electric or other suitable type of furnace. The molten mass may be allowed to cool and crystallize, whereby it becomes somewhat like corundum in its physical characteristics, especially with reference to its 105 hardness. This material after crystallization or cooling is crushed and the resulting granules are graded, so that the proper sizes, as considered desirable, may be obtained for use.

110 Since the non-slipping characteristics of the tread block will depend to some extent upon the size of the granules, I utilize that size of grain which is deemed the most 115 suitable for the particular location in which the block is to be placed. While various sizes of grain may obviously be used, I prefer grains which will pass through a 60 mesh sieve or even finer, since this material 120 125 130

will not have large destroying or abrading effects upon shoe leather and will be large enough to prevent slipping.

Owing to the ease with which this tile 5 may be placed and held in position if laid in cement, I preferably so shape and construct the tile that it may be used in combination with a cement flooring. Heretofore, it has not been feasible to lay a 10 safety tread merely by embedding a block of anti-slipping material in cement, so elaborate constructions have necessarily been provided to hold the tread in place.

Referring to Fig. 1, I have there illustrated one form which a tile may be given, this particular shape being adapted for a stair tread or a flooring edge, as on a platform near a car track. As illustrated, the tile is a flat plate 1 having a continuous 20 plane surface 2 for the tread, a rounded nose 3 on the upper front corner where wear is most likely to occur, and a dovetail portion 4 having beveled edges 5 at the rear to interlock with a concrete construction to 25 hold the tile in place. Other suitable shapes may obviously be employed to engage the cement or other means employed to hold the tile in place.

In order to place this tile on a railroad 30 platform, for example, I provide a cement foundation 6 and embed a row of the safety blocks 1 at the forward edge of the walking surface. The tile is sunk into the flooring or cement is placed in the rear thereof, so 35 that the surface 2 of the tile is flush with and in the same plane with the cement surface 7 of the platform. In this manner, I provide a smooth continuous plane for a tread surface, which will in no way interfere with walking or the wheeling of trucks 40 thereover, and which will resist wear for a long period of time and remain uniform in its characteristics for preserving the safety of pedestrians.

45 I claim as my invention:—

1. An anti-slipping tread block comprising anti-slipping particles of a hardness of 50 9 or more and a ceramic vitrified bonding material holding said particles together in a unitary wear resisting structure, said particles constituting a major portion of the block and receiving substantially all of the traffic wear.

2. An anti-slipping tread block comprising 55 a body of wear-resisting, anti-slipping granules unitarily bonded by vitrifiable clay material fused into intimate contact with the grains, said bond being hard, durable and capable of resisting the tendency for 60 frictional wear to strip said granules from the surface of the block and disrupt its structure and said block having a high frictional coefficient permitting only a slight degree of slippage and affording thereby an 65 easy walking tread surface.

3. A safety tile comprising anti-slipping, wear-resisting grains integrally united into a porous structure by a vitreous ceramic bond prefused into intimate contact with the grains and forming a durable body in which 70 the grains constitute the major portion of the bonded mass and receive substantially all of the traffic wear.

4. An anti-slipping tile comprising crystalline granules of a hardness of 9 or more 75 and a vitrified, glassy clay material bonding said granules into a porous, wear-resisting structure having an imperforated, continuous, rough surface capable of preventing a 80 pedestrian slipping thereon.

5. A tile comprising wear-resisting, anti-slipping granular material of a hardness of 9 or more and a proportionately small amount of a vitrified, glassy ceramic bond unitarily united as a dense porous structure 85 of high tensile strength, which has an imperforated and continuous tread portion consisting mainly of said granular material and being capable of resisting wear and preventing slipping of foot gear thereon. 90

6. An anti-slipping tile comprising grains containing crystalline alumina bonded into a hard, wear resisting body by a vitrifiable ceramic material fused into intimate contact with the grains, which is capable of resisting the normal abrading action of foot-wear tending to disrupt the bond, fracture the grain and dislodge particles thereof from the tile. 95

7. A safety tile comprising crystalline 100 alumina grains bonded by a vitrified, glassy ceramic material into a porous mass, said grains constituting the major portion of the body and permanently forming an anti-slipping tread surface under all conditions of 105 wear, and said bond uniting integrally with the surfaces of alumina crystals.

8. A safety tread comprising a flat plate of previously fused alumina grain bonded by a relatively small amount of a glass 110 fused clay material, said plate being dense, hard, rough surfaced, wear resistant and anti-slipping to footgear and having an imperforated, continuous, plane top surface 115 consisting substantially wholly of alumina grains which offers no obstructions to traffic and may be easily cleaned and maintained in a sanitary condition.

9. An anti-slipping tile comprising small crystalline granules of hard, wear-resisting 120 material constituting the major portion of the tile and a relatively small amount of bond containing a low fusing clay material fired to a unitary mass.

10. An anti-slipping tile comprising crystalline material of a hardness of 9 or more 125 which will pass through a 60 mesh sieve and a low fusing clay material containing slip clay fired to a glassy condition and bonding the crystalline material into a du- 130

- rable mass, said crystalline material constituting the major portion of the tile surface and receiving substantially all of the wear.
11. An anti-slipping tile comprising small sized crystalline alumina grains and a ceramic bond containing a low fusing material fired to a dense vitreous mass and uniting separated grain surfaces, pores being interspersed with the bond masses between
- 10 the grains and said alumina constituting the major portion of the tread and receiving substantially all of the traffic wear.

12. An anti-slipping tile comprising small sized crystalline alumina granules and a lesser portion of a glass-fused bond therefor containing slip clay, feldspar and ball clay, said tile being dense, porous and having a tread surface consisting mainly of the alumina granules.

Signed at New York, N. Y., this 25th day of April, 1918.

HERBERT K. DODGE.